

April 26, 1927.

1,625,888

J. H. GILLIS

ROOFING ELEMENT AND METHOD OF MAKING THE SAME

Filed Aug. 15, 1923



Patented Apr. 26, 1927.

1,625,888

# UNITED STATES PATENT OFFICE.

JULIUS H. GILLIS, OF ELIZABETH, NEW JERSEY, ASSIGNOR, BY MESNE ASSIGNMENTS,  
TO ANACONDA SALES COMPANY, A CORPORATION OF DELAWARE.

## ROOFING ELEMENT AND METHOD OF MAKING THE SAME.

Application filed August 15, 1923. Serial No. 657,489.

This invention relates to roofing elements and processes for making the same, and has to do primarily with roofing elements in the form of boards, strips, tiles, single or multiple shingles, and the like. These elements are of the composite type and consist of a base formed of various materials well-known in the art under the general name of roofing compositions, and a protective metallic layer or coating applied to the base to form a weather surface therefor.

Composition roofings are in wide use at the present time, and serve to replace roofing materials hitherto used, such, for instance, as wooden shingles, slate, etc. These composition roofings are formed of paper, felt, burlap, or similar materials, impregnated with water-proofing materials such as bituminous substances, magnesite compositions, and various other non-hygrosopic, heat insulating materials held together with a suitable binder. Such composition roofing material is used in a variety of forms, as, for instance, strips, single or multiple shingles, tiles, etc. The multiple shingles consist of a strip of roofing of appropriate dimensions having an indented edge so formed that when these elements are laid in courses in the usual manner the indented edge is exposed so as to give the usual appearance of a shingle roof.

Composition roofings of the type above generally referred to have numerous advantages, due to their comparatively low cost, easy method of application, and heat insulating qualities. However, when such elements are laid in place on the roof in overlapping courses the exposed portion is likely to warp or curl, and after periods of use the composition deteriorates due to the volatilization of the oils used in their manufacture. Also such composition materials are not altogether pleasing to the eye.

Roofing in the form of sheets or strips of metal has also been in common use for some time, and while such metallic roofing has a long life and may be given a distinctive and attractive appearance, the high heat conductivity of the metal makes such roofing objectionable. Also the cost of metallic roofing is much higher than that of the composition type and this cost is increased owing to the necessity of providing heavy insulating sheathing beneath it.

A composite roofing element devised to

combine the advantages of the two types previously referred to, is shown and described in the Patent No. 1,449,058, granted March 20, 1923, to Thomas Robinson. This element consists of a composition base of various forms, prepared by methods which are well known. On that surface of the element which is to be exposed to the weather, there is applied a thin coating of a non-corrodible metal, such, for instance, as copper or zinc. This metallic coating is limited to the weather surface of the element and it serves to stiffen the base to prevent warping and curling, to protect the relatively soft base materials, and to prevent deterioration caused by volatilization of the base oils. By using a thin layer of metal and by limiting this layer to the weather surface of the element, the cost of the new type of roofing is but little greater than that of the unprotected base and such elements may be laid as easily as ordinary composition roofings and without that degree of care which is necessary in the case of metallic roofings to prevent leaks. In the patent above referred to the metal coating is applied directly to the surface of the base in various ways, as for instance, by electrodeposition. In the co-pending application of Thomas Robinson, Ser. No. 618,246, filed February 10, 1923, there is shown and described a somewhat similar element which is given an attractive appearance by the application of a layer of granular material such as crushed slate or crushed petroleum coke pressed into the surface of the base before the metallic layer is applied. Also in the co-pending application of Thomas Robinson, Ser. No. 652,563, filed July 19, 1923, there is shown and described a process for making elements which consist of a base and a preformed metallic layer which is applied thereto by pressure. In this particular process the base is of ordinary composition and may have either a plain or granular surface to which a preformed metallic layer or coating, cut to the appropriate size and shape, is applied by the application of pressure sufficient to cause the metal to conform to the irregularities of the base and adhere thereto.

The present invention is intended to improve the quality of the roofing elements made by either the electrolytic or pressure processes, above referred to, and is intended

further to provide a process by which there is secured a stronger adherence between the metallic coating and the base. It is adapted especially for use with electrolytic processes 5 for applying the coating for in such processes it will be clear that it is necessary to give the base a coating of electrical conducting material before the metal is applied thereto. The conducting material which is 10 ordinarily used for this process is powdered graphite, which is held in place by the use of a suitable adhesion. In preparing the elements for the deposition of the metal their weather surfaces are sprayed or otherwise 15 treated with an adhesive which may take the form of a saturated solution of asphalt in carbon tetrachloride. A layer of powdered graphite is then dusted or brushed thereover and when the adhesive dries the 20 graphite is firmly held in place. This conducting coating is necessary for the electrolytic processes in which the metal is deposited over the coating in such a way as to conform to the irregularities of the base 25 so that a good binding effect is produced. However, it sometimes happens, due to carelessness on the part of the workman, that the conducting material is applied unevenly or in a much thicker layer than is necessary 30 for carrying on the deposition, and if too thick a layer of graphite, which has lubricating qualities, is applied to the base lying between it and the metallic layer extreme changes in temperature causing expansion 35 and contraction of the metal, may result in loosening this layer from the base.

The object of the present invention may be restated then, as the provision of a process 40 by means of which the metallic layer is bound firmly directly to the base even though there is an intervening coating of conducting material and this process improves the quality of the roofing even in those cases where the layer is applied by 45 pressure and no conducting material intervenes between the metal and the base. In carrying out the process, I take advantage of the fact that the base contains a plastic substance which softens and expands upon 50 heating and I heat the metallic coating after the latter has been applied to the base either by pressure or deposition, confining this heat to the metal in such a way that only a thin stratum of the base immediately underlying 55 the coating is heated by conduction. This application of heat causes the plastic material on and in the base to soften and swell and during this heating I apply pressure to the metallic layer so as to cause the softened plastic material to wet the layer over 60 all its surface in contact with the base. The heat is applied and regulated in such a way that the base itself is not heated throughout its thickness and I prefer to apply the heat rapidly and to regulate the pressure so

as to give the desired effect without softening the base so that the element cannot be readily handled.

In order to secure a good bond between the base and the layer I prefer to use a base 70 which contains asphalt as an ingredient although other similar materials used for binders in the past are also satisfactory. The new process, however, is applicable in connection with any type of base, whether 75 or not it is impregnated with asphaltic material, although in the latter case it is preferable to use an adhesive containing asphalt for binding the conducting coating to the base. If no conducting coating is to be 80 used, as in the case of preformed metallic layers applied by pressure, then it is preferable to apply a thin film of asphalt or similar material to the base before the metal is pressed in place thereon. 85

In taking advantage of the plastic material on and in the base for causing the layer to adhere thereto, there are several essentials which must be borne in mind in connection with the heating step. I have found that the bond is the stronger, the hotter the layer is made, but in applying this heat it should be limited to the layer because if the heat enters the base to any great extent, it is likely to cause volatilization of the oils and to soften the base and render it flexible so that the elements after the heating cannot be readily handled but must be stored and allowed to cool in such a way that they will not warp. Again it is necessary that the heat should be uniform throughout the metallic layer, otherwise bulging of the layer is likely to occur with the result that when the source of heat is removed the layer will not conform properly to the surface of the element. It is also necessary that the heating should be carried on rapidly and that the layer should be raised to a temperature sufficient to soften the plastic material in the base only to a very slight depth. The longer the heat is applied, the greater will be the layer of the base which is softened, and while it is only necessary to heat the plastic material in a thin stratum of the base in order to secure a firm bond, slow heating 105 does not improve the quality of the bond but on the other hand causes the heat to be conducted into the base so that it is softened. The application of pressure during the heating improves the quality of the bond but such heat and pressure cannot be carried on by any of the ordinary methods such as by passing the elements through steam or gas heated rolls because the heating so produced is too slow. Also it is not possible to carry on the heating by the application of flames directly on the metal, inasmuch as such treatment results in the deposition of combustion products on the metal 110 injuring its appearance and in some cases 115

causing a slight corrosion. Heating by flame also has the disadvantage that it is almost impossible to secure an even and uniform application of heat, and, as has previously been explained, this results in bulging of the layer.

I have found, however, that application of heat with the desired rapidity under the proper regulation and without the several other disadvantages of hot roll or flame heating, may be carried on by making use of the heating effect of the electric current. For this purpose I use presses or rolls provided with suitable contacts which cause a current of the desired intensity to flow through the metallic layer. This rapidly generates heat which is localized and confined in the layer and which does not spread to any appreciable extent into the base. By properly regulating the current the heating operation may be carried on economically and with great rapidity, and the elements which have been subjected to the application of heat and pressure may be easily supported in a way which prevents warping or curling of the base or bulging of the layer. Also by generating heat in the layer itself there is no possibility of the layer bulging or expanding away from the base. Various mechanical devices may be used for carrying on the present process, but in the accompanying drawings I have illustrated various forms of mechanism which are satisfactory for such purposes. In these drawings,

Fig. 1 is a cross-sectional view of a smooth surface element showing the metallic layer applied thereto,

Fig. 2 is a view similar to Fig. 1, but showing the metal applied over the granular surface,

Fig. 3 is a plan view of a multiple shingle element showing the outline of the coating and location of the contacts,

Fig. 4 is a view similar to Fig. 3, showing the modifications necessary in connection with a single shingle element,

Fig. 5 is a view similar to Fig. 3 but showing the contacts in modified form,

Fig. 6 is a diagrammatic view in side elevation of a pressure device provided with contacts,

Fig. 7 is a plan view of a flashing strip having a metallic coating,

Fig. 8 is a view in side elevation of a modified form of device for treating such strips,

Fig. 9 is a cross-sectional view of a detail of the pressure rolls used,

Fig. 10 is a phantom view of one of the rolls showing the current paths.

Referring now to the drawings, the roofing element is seen to consist of a base 11, provided with a metallic coating 12, extending over the weather surface of the base and

applied in such a way as to conform to the irregularities thereof. In the element shown in Fig. 1, the base is illustrated as having irregularities which are shown somewhat enlarged for purposes of illustration. It will be understood that the presence of these irregularities improves the mechanical bond between the base and metal, as set forth in the Robinson Patent, No. 1,449,058, above mentioned. If suitable materials are employed for the base, its surface will have natural irregularities sufficient to give the desired bonding effect, or the base may receive a layer of granular material, as by coating the base with a film of asphalt and embedding granular material, such as slate, therein, as described in the Robinson application, Ser. No. 618,246, above referred to. This granular material gives the rough irregular surface over which the metal is to be applied. In Fig. 2 the base is shown to be provided with a granular layer 13, disposed over the surface thereof. This granular layer, as has previously been explained, may consist of crushed slate or crushed coke which has been pressed into the surface of the base while the latter is still soft. The element illustrated in Fig. 2 has a metallic layer 12, applied over these granules in such a way as to enter the interstices between the granules and so conform to the irregular surface. In Fig. 3 the element 14 is of the multiple type and one edge is provided with cut-outs 15 which serve to define three separate shingles 16. 100

These cut-outs are formed so that when the multiple element is laid in place only the projecting portions defined by the cut-outs are exposed, and a roof formed of multiple elements has the usual appearance of an ordinary shingle roof. In this form of element each of the shingles defined thereon is provided with a metallic layer 16, terminating at the rear end in a neck 17 which is extended so as to underlie the cut-out of

the shingle of the overlying course. With this arrangement it will be seen that all the exposed portions of the shingle are covered with metal so that to all intents and purposes the roofing may be considered to be a continuous metallic roofing. The element illustrated in Fig. 4 is a single shingle of the usual outline having a coating 18 which terminates in a triangular portion

19 which serves to underlie the space between adjacent elements of the overlying course. As these shingle elements are usually laid by hand the portion which underlies the space between the elements of the next course above is made somewhat greater than the neck 17 so as to allow for carelessness of the workmen in applying the shingles.

The new process may be practiced without regard to the particular shape and size 130

of the roofing elements to be treated, but slight modifications are necessary in the construction of the presses or rolls as the case may be, and also in the location of 5 the contact members, according to the outline of the elements and the shape and size of the metallic layer thereon. For convenience the elements have been shown in a form which is widely used at present, and the 10 necessary contacts and electrical connections are designed for use with such elements, but it will be understood that the general principles here set forth are applicable regardless of the particular outline which the 15 elements have.

Referring now to Fig. 6, the press which I make use of has a bed 20, the working face of which is preferably provided with a layer 21 of yielding material, such as 20 rubber. Mounted above the bed is a movable plunger 22, which may be mounted to move in a standard in accordance with the usual press construction. The face of this plunger is provided with a yielding cushion 25 surface 23 which may be made of rubber suitably treated to withstand the temperatures which are to be employed. This rubber cushion will be preferably secured in place in the plunger in any convenient way, 30 so that it may be readily removed and replaced when occasion demands. Secured in the face of the plunger and insulated from the body thereof, are spaced contacts, these contacts lying flush with the surface of the 35 cushion so that when the plunger is depressed against an element laid on the bed the contacts will strike the face of the element while pressure is exerted through the cushion to hold the metallic layer of the 40 element firmly against its base. It will be understood that the shape and size of the plunger will depend upon the shape and size of the element which is to be treated, and the spacing of the contacts in the face 45 of the plunger will also depend on the form of the metallic layer which has been applied to the element base. In Fig. 3 there are shown contacts suitable for a multiple element which consists of three shingles 50 united along their rear edges. Located in the face of the plunger are spaced contacts 25 which will engage the metallic layer of the element along its rear edge where the neck portion joins the body of the layer. 55 Contacts 26 serve to engage the front edge of each layer and the curved contacts 27 are spaced so that when the plunger is depressed these contacts will engage the end of the neck portions. The contact 25, as is 60 illustrated in the right of Fig. 3, is connected to one terminal of a source of power and the current accordingly enters the contact 25 and spreads in both directions through the metallic coating being taken off 65 through contacts 26 and 27. These con-

tacts are then joined by a conductor 28 which lies within the face of the plunger and the conductor 28 is in turn connected to the contact 25 for the next metallic layer. The current spreads through this layer as 70 before, passes out through contacts 26 and 27, and enters the central contact 25, being finally taken off by means of a conductor 29 which connects the contacts 26 and 27 for the layer at the left in Fig. 3. This 75 conductor is then connected to the other side of the line. It will be clear that when the contacts are out of engagement with the layers of the element no current will flow but immediately upon depression of the 80 plunger into contact with the element current will flow through the metallic layers, as has been explained.

The contacts illustrated in Fig. 4 have been designed to take care of the particular 85 form of metallic layer used in a single shingle. There is a central contact bar 30 across the layer at the base of the triangular portion, an annular contact 31 which engages the layer at the apex and another 90 contact 32 which engages the front edge of the layer. The current paths are similar to those previously described, the current entering through the central contact and spreading through the layer, to be taken off through the contacts 31 and 32. In Fig. 5 there is shown a somewhat modified layout for the contacts which shows the use of conductors within the face of the plunger. 95 In this arrangement there is provided a contact 33 which engages one metallic layer along the top edge and along the side of the neck portion. Another contact 34 extends along the front edge of one layer, then rearwardly to overlie the edges of adjacent layers, then along the edge of the second layer, 100 and up and around the neck portion, as before. Contacts similar to 34 are used in any number desired, depending on the number of shingles in the element, and the current is then removed through a contact 35 which extends along the front edge of one layer and rearwardly along its side. In this arrangement current will enter contact 105 33 and travel through the metallic layer to the contact 34, passing through the contact to the next layer, thence through the layer to the next contact 34, and thence out through contact 35. The contacts are so designed that current will flow through all 110 portions of the metal layer, heating it evenly and uniformly.

In Fig. 7 there is illustrated a form of roofing material useful for flashing strips. 115 This consists of a long strip of base material having a facing of metal and for applying heat and pressure to such a strip I have found it convenient to make use of pressure rolls provided with electrodes on the surface thereof. Such an arrangement is illustrated 120 130

in Fig. 8. At one end of the apparatus is a pair of rolls 36 and 37. The lower roll 37 is an ordinary steel roll mounted to revolve freely in fixed bearings. The upper roll 36 5 may be of rubber, as illustrated at 38 in Fig. 9, or may be a steel roll provided with a rubber surface. At either end of this roll is a ring electrode 39, lying flush with the face of the roll. These electrodes may be 10 connected to a suitable source of power by means of brushes or other contact arrangements and are designed so that the current enters one contact 39 of Fig. 10, and passes out the other 40. The current passing be- 15 tween the electrodes will accordingly travel through the metallic layer on the strip and in its passage will spread through paths as illustrated at 41 in Fig. 10. The strip 42 is shown to enter the pressure rolls from the 20 left in Fig. 8, passing through contact rolls 36, 37 and then passing through a series of rubber pressure rolls 43, which exert regulated pressure on the strip. The current may be so selected that the heating will be carried 25 on rapidly and the strip is moved with a steady uniform movement through the rolls. If it is desired to increase the rate of heating it is possible to make use of a series of contact rolls 36, 37, as shown at the right in 30 Fig. 8, the strip moving from these rolls being later subjected to pressure between rollers similar to those illustrated at 43. In its passage through the rolls the metallic layer is heated by the current travelling be- 35 tween the electrodes and pressure is applied not only by the electrode rolls but also by the succeeding rubber pressure rolls, so that when the strip emerges from the apparatus the binding of the metal to the base is com- 40 plete. It is necessary that the pressure rollers 43 should be spaced and aligned in such a way as to maintain the strip in its straight condition without sagging or bending until the plastic material which has been caused 45 to wet the metal during the heating has set, as otherwise the metal might pull away from the base and the desired adherence be lost.

I have found that a satisfactory bond is se- 50 cured by heating the copper to approximately 350° F., although the degree of heat will naturally depend on the character of the plastic material which serves to produce the bond. The particular degree of heat above referred to has been found satisfactory in the 55 case of an element to which the metallic layer has been applied by electro-deposition over a thin film of graphite held in place by an adhesive containing asphalt. The pres- 60 sure required in the above example is approx- 65 imately 25 pounds per square inch and I have also found that a current of approx- 70 imately 150 amperes per inch of width of the coating is about the most satisfactory intensity. The voltage required to produce such 75 a current in this particular type of element

is approximately one half a volt for contacts which are five inches apart, and the application of such a current for a period of twenty seconds produces the desired heating effect.

I have found that the application of heat 70 as above described causes the plastic material of the base to expand and swell with a slight bubbling effect which causes this softened material to wet the under surface of the metal. Where the metal has been applied by electrolysis it has been found that this plastic material permeates the conducting layer with the result that this layer is absorbed in the base and accordingly does not intervene between the surface of the base 80 and the metal. This is particularly true where the conducting layer is graphite which has been caused to adhere to the base by means of an adhesive containing asphalt.

The process above described results in a 85 thorough binding of the metal to the base throughout the surface of the metal and is applicable whether the metal has been applied by electro-deposition or by pressure. In the first case, however, it has the advantage of causing the conducting material to be absorbed into the base and this is of peculiarity advantage where graphite is used owing to the lubricating qualities of the graphite. The process, however, is of equal application where the performed layer is applied by pressure and is also capable of application to roofing elements made in accordance with the process disclosed in the co-pending application of Thomas Robinson, Ser. No. 606,339, filed Dec. 11, 1922, wherein the metal is applied in the form of a fine powder bound to the base by a suitable adhesive.

The generation of the heat in the metallic layer not only serves to confine and localize the heating effect so that the base is not rendered flexible, but the element may be readily handled at the completion of the process, since the heat does not extend into the base to any appreciable extent. I have 105 also found that this application of localized heat has another incidental advantage inasmuch as the heating is carried on under those conditions which are best for annealing the metal layer. This results in improving the quality of the metal, as well as producing a more perfect bond.

The contacts which are used for causing the current to flow through the metal may 110 be of copper, iron, or nichrome, and will last indefinitely. Also the cushion which is applied to the face of the plunger and to the rollers may be made of rubber of such characteristics that it will readily withstand the degree of heat required and since this heat is of comparatively low temperature and is applied for a comparatively short length of time, the cushions will last for an indefinite period. It will accordingly be 115 seen that the process is relatively inexpen- 120 125 130

sive to carry on and the bond between the metal and the base is not produced by added materials but by materials which are present in the base or necessarily applied thereto in connection with the application of the conducting material.

It will be understood that the moving plunger in the press is preferably power-driven, and is arranged so that the pressure to be exerted by it may be regulated. The simplest form of press will be provided with a single plunger of such size as to act on a single element at a time. Ordinarily a plunger arranged to act on a four-shingled unit will be the maximum size used, although multiple shingle units may be treated in a single unit press, pressure being exerted successively on each of the shingle coatings. Ordinarily it is most convenient to arrange the presses in pairs so that one workman can feed roofing elements to them in alternation, and the time required for the application of heat is just about sufficient for placing a new element in the press and starting the heating operation. From the presses the elements are conveyed to storage-warehouses or shipping platforms and since the metal layer is comparatively thin it will radiate heat with such rapidity that the elements may be handled by the workman as soon as they are removed from the press. Also the elements are not appreciably softened during the heating operation, and it is not necessary to permit them to cool off before they are handled.

I claim:

1. A method of making roofing elements, which comprises preparing a base containing a plastic substance, allowing the plastic substance to assume a non-adhesive condition, applying a metallic layer to the surface of the base, and simultaneously heating the metal and pressing it against the base, the heating of the metal being carried on to an extent sufficient to soften the plastic substance and render it adhesive.

2. A method of manufacturing roofing elements, which comprises preparing a base containing a plastic substance and having an irregular surface, allowing the plastic substance to assume a non-adhesive condition, applying a metallic layer over the irregular surface of the base in such manner as to conform to the irregularities thereof, and simultaneously heating the metal and pressing it against the base, the heating of the metal being carried on to an extent sufficient to soften the plastic substance so that it wets and adheres to the metal.

3. The method of manufacturing roofing elements, which comprises preparing a base containing a plastic substance, allowing the plastic substance to assume a non-adhesive condition, applying a metallic layer to the surface of the base, pressing the

layer of metal against the base, and, while the metal and base are so held, generating heat in the layer sufficient to cause the plastic substance in the base to soften and adhere to the under surface of the metal.

4. The method of manufacturing roofing elements, which comprises preparing a base containing a plastic substance, allowing the plastic substance to assume a non-adhesive condition, applying a metallic layer to the surface of the base, and passing an electric current through the layer to heat the latter to an extent sufficient to soften the plastic substance to cause it to wet the layer and adhere to it.

5. The method of manufacturing roofing elements, which comprises preparing a base containing a plastic substance, allowing the plastic substance to assume a non-adhesive condition, applying a metallic layer to the surface of the base, pressing the base and layer into intimate contact, and, while the base and layer are so held, causing an electric current to flow through the layer to raise the temperature of the latter to an extent sufficient to soften the plastic substance and render it adhesive.

6. The method of manufacturing roofing elements, which comprises preparing a base containing a plastic substance, allowing the plastic substance to assume a non-adhesive condition, applying a conductive material to the surface of the base, electrodepositing a metallic layer over the conducting coating, holding the layer and base in intimate contact, and heating the layer to an extent sufficient to soften the plastic substance and render it adhesive.

7. The method of manufacturing roofing elements, which comprises preparing a base containing a plastic substance, electrodepositing a metallic layer on the surface of the base, pressing the base and layer into intimate contact, and, during the pressing operation, generating heat in the metallic layer to raise its temperature sufficiently to soften the plastic substance to cause it to wet and adhere to the metal.

8. The method of manufacturing roofing elements, which comprises coating a base with a film of asphalt, allowing the asphalt to cool and harden, applying a metallic layer over the asphalt coating, pressing the base and layer into intimate contact, and, during this operation, generating heat in the layer sufficient to soften the asphalt coating to cause the latter to wet and adhere to the under surface of the metal.

9. The method of manufacturing roofing elements, which comprises coating a base with an asphaltic film, allowing the film to cool and harden, applying a conducting coating over the film, electrodepositing a metal layer over the conducting coating, and generating heat in the layer to raise

its temperature sufficiently to cause it to soften the asphaltic film so that the latter adheres to the metal.

10. The method of manufacturing roofing elements, which comprises preparing a base containing a plastic substance, allowing the plastic substance to assume a non-adhesive condition, applying a conducting coating to the base, electrodepositing a metallic layer over the coating, and heating the layer to cause it to soften the plastic material to an extent sufficient to cause the layer to absorb the conducting coating and wet and adhere to the layer.

15. 11. The method of manufacturing roofing elements, which comprises preparing a base containing a plastic substance, allowing the plastic substance to assume a non-adhesive condition, applying a metallic layer to the 20 surface of the base, and progressively uniting the base and layer by generating heat in the layer while it is in position on the base, the heating being carried on to an extent sufficient to soften the plastic substance and 25 render it adhesive.

12. The method of manufacturing roofing elements, which comprises preparing a base containing a plastic substance, allowing the plastic substance to assume a non-adhesive 30 condition, applying a metallic layer to the surface of the base, and uniting the base and layer by progressively pressing the base and layer into contact and simultaneously generating heat in the metal to an extent 35 sufficient to soften the plastic substance and render it adhesive.

13. The method of manufacturing roofing elements, which comprises preparing a base containing a plastic substance, allowing 40 the plastic substance to assume a non-ad-

hesive condition, applying a metallic layer to the surface of the base, and uniting the base and layer by progressively pressing the layer into contact with the base and causing an electric current to flow through the layer 45 along a path moving throughout the length of the layer, the current raising the temperature of the metal to an extent sufficient to cause it to soften the plastic material and render it adhesive. 50

14. The method of manufacturing roofing elements, which comprises preparing a base containing a plastic substance, allowing the plastic substance to assume a non-adhesive condition, applying a metallic layer to the 55 base, and passing the base and layer through pressure rolls and causing an electric current to flow through the layer along the line at which the maximum pressure is exerted, the current raising the temperature 60 of the metal to an extent sufficient to soften the plastic material and render it adhesive.

15. A roofing element which comprises a base coated with a plastic substance, a conducting coating over the plastic coating, 65 and an electrodeposited metallic layer over the conducting coating and bound to the base in part by the plastic substance which adheres to the under surface of the metal.

16. A roofing element which comprises a 70 base coated with an asphaltic compound, a coating of graphite on the surface of the base, and an electrodeposited metallic layer over the graphite, the metallic layer in part adhering to the graphite and in part being 75 held to the base by means of the asphaltic compound which contacts with the under surface of the metal and adheres thereto.

In testimony whereof I affix my signature.  
JULIUS H. GILLIS.